

## 1

3,111,465  
ELECTRODEPOSITION OF COPPER AND  
COPPER ALLOYS

Frank Passal, Detroit, Mich., assignor, by mesne assignments, to M & T Chemicals Inc., New York, N.Y., a corporation of Delaware  
No Drawing. Filed Feb. 9, 1959, Ser. No. 791,824  
17 Claims. (Cl. 204—44)

The present invention relates to the electrodeposition of decorative and protective copper and copper alloys from improved alkaline-cyanide type baths. The present application is a continuation-in-part application of U.S. Serial No. 666,766 and No. 666,784, both filed June 19, 1957, issued as U.S. Patent Nos. 2,873,234 and 2,873,235, respectively.

The object of this invention is to provide improved baths for the electrodeposition of copper and copper alloys.

Another object of this invention is to provide an improved process for electrodepositing copper and copper alloys.

The present invention contemplates electrodepositing decorative and/or protective copper or copper alloys from alkaline-cyanide baths containing between 0.01 and 0.2 g./l. (grams per liter) of N-substituted  $\beta$ -alanines selected from the class of compounds having the following two general structural formulae:

- (1)  $R(H)NC(R')HCH_2C(O)OX$ , and  
(2)  $RN[C(R')HCH_2C(O)OX]_2$

wherein R is an alkyl radical having from 8 to about 16 carbon atoms in the chain; R' is a group selected from hydrogen and alkyl radicals having 1 to 4 carbon atoms (preferably hydrogen); and X is a cation selected from the class consisting of hydrogen, sodium, potassium, calcium, lithium, magnesium and ammonium ions (preferably sodium or potassium). The alkyl radicals (R) are generally derived from long chain natural alcohols, the preferred natural product being the coconut derivative, generally called "coco," which is predominantly a  $C_{12}$  natural product. The alkyl radicals having between 12 and 14 carbon atoms in the chain are preferred. These  $\beta$ -alanines are usually available in the form of the sodium or the potassium salts which are preferred compounds for use in the present invention. The salts of the other cations noted hereinbefore are also useful, as are the free acids where care is taken to vent HCN evolved. The amino type material, Formula No. 1 hereinbefore, is preferred to the imino type material, Formula No. 2 hereinbefore. This preference is based on its somewhat more advantageous solubility and adsorption characteristics. Although baths may contain these  $\beta$ -alanines in amounts between 0.01 to 0.2 g./l. it is preferred to use amounts between 0.04 and 0.09 g./l.

The preferred  $\beta$ -alanines of this invention have the following general structure:  $RNHCH_2CH_2COONa$  (an alkyl  $\beta$ -amino propionate), and  $RN(CH_2CH_2COONa)_2$  (an alkyl  $\beta$ -imino dipropionate). They are stable in the electrolyte and even impart some brightening action. A compound of this class which has been successfully used is the sodium salt of a coconut alcohol derivative of  $\beta$ -amino propionate.

The N-substituted  $\beta$ -alanines are useful in a wide variety of cyanide type baths containing excess potassium or sodium cyanide (herein called "free cyanide") and

## 2

processes for the plating of copper and copper alloys. These generally include the following:

- (1) Copper "strike" baths:  
Copper..... About 15 g./l.  
Free potassium or sodium cyanide..... 11-15 g./l.  
Temperature..... 48°-60° C.  
Agitation..... Little or none.  
Current density..... 10-50 a.s.f.
- (2) Intermediate speed baths:  
Copper..... 30-38 g./l.  
Free potassium or sodium cyanide..... 7.5-15 g./l.  
Potassium or sodium hydroxide..... 15-30 g./l.  
Potassium or sodium carbonate (optional)..... About 15 g./l.  
Temperature..... Generally 65°-82° C.  
Agitation..... Yes.  
Current density..... 10-80 a.s.f.
- (3) Bright copper baths:  
Copper..... 37-75 g./l.  
Free potassium or sodium cyanide..... 3.7-15 g./l.  
Potassium or sodium hydroxide..... 15-30 g./l.  
Brightener, e.g., selenium bis diethyldithiocarbamate..... About 0.004 g./l.  
Temperature..... Generally 65°-82° C.  
Agitation..... Yes.  
Current density..... 5-50 a.s.f.
- (4) Brass plating baths:  
CuCN..... 30-225 g./l.  
Zn(CN)<sub>2</sub>..... 9.4-71 g./l.  
Total NaCN..... 56-425 g./l.  
Na<sub>2</sub>CO<sub>3</sub>..... 30-123 g./l.  
Free NaCN..... 30-225 g./l.  
Temperature..... 20°-38° C.  
Current density..... 2-20 a.s.f.
- (5) Bronze plating baths:  
Tin (as stannate)..... 11-16 g./l.  
Copper..... 18-30 g./l.  
Free KCN or NaCN..... 20-25 g./l.  
Free KOH or NaOH..... 6-10.6 g./l.  
Temperature..... 62°-71° C.  
Current density..... 20-100 a.s.f.

These baths and operating conditions are merely illustrative of plating from alkaline-cyanide type copper and copper alloy baths. Alkaline-cyanide baths and processes are described in "Modern Electroplating," edited by A. G. Gray, pages 98-114 and 194-225 (1953). Electroplating from the bronze and brass plating baths illustrated may utilize the respective alloy anodes or copper anodes with periodic additions of the tin or zinc salts as they are depleted. Other additives of the type commonly used with alkaline-cyanide type baths are generally used in conjunction with the  $\beta$ -alanines of this invention. These include such additives as citrates, tartrates, or saccharates, and the metallic brighteners, organic brighteners, etc.

When the baths of the present invention contain such brighteners as lead, selenium, tellurium or thiocyanate, and the  $\beta$ -alanines, it is found that the  $\beta$ -alanines actually impart additional brightening characteristics to the bath, thus they function as a cooperative brightener. Their

primary function is as an anti-pitting agent. They also tend to make the bath more tolerant to impurities.

As is generally known in electrodeposition from alkaline-cyanide baths best results are usually achieved when the process utilizes a method of preventing the thin film immediately adjacent the cathode from becoming depleted in metal ion content. This is conventionally accomplished by agitation such as solution pumping, cathode movement, air agitation, or by diffusion effects, e.g., current interruption, periodic reversal, etc., or, by combinations thereof. The use of air agitation is generally not preferred in baths containing the N-substituted  $\beta$ -alanines. Their action on the bath is such that the bath is characterized by a relatively stable foam. When air agitation is used the foam blanket is likely to grow to high. However, under particular conditions this might be acceptable although generally it is preferred to use one of the other methods, e.g., cathode movement or solution pumping, to achieve the results desired.

For the purpose of providing a better understanding of this invention, examples of various baths and process conditions are summarized in Tables I and II; Table I illustrating copper plating, and Table II illustrating bronze plating.

Many wetting agents are not effective in alloy plating in that they tend to vary the alloy composition. These  $\beta$ -alanines do not effect the alloy composition, particularly in bronze plating. In addition, they tend to act as brighteners (in conjunction with metallic brighteners) in bronze plating.

The sound copper and copper alloy electrodeposits obtained from alkaline-cyanide type baths of the present invention are obtained on such conventional basis metals as iron, steel, nickel, zinc, lead, copper, etc., and alloys thereof. On certain basis metals such as iron or steel and zinc-base die castings the basis metal is first given an initial thin flash of copper from a low efficiency cyanide copper bath.

As many embodiments of this invention may be made without departing from the spirit and scope thereof, it is to be understood that the invention includes all such modifications and variations as come within the scope of the appended claims.

I claim:

1. An improved alkaline-cyanide bath for plating a metal selected from the class consisting of copper and copper base alloys which comprises copper cyanide, free cyanide, and between 0.01 g./l. and 0.2 g./l. of at least

Table I

| Constituent in g./l. or Plating Condition            | 1    | 2    | 3   | 4     | 5     | 6     | 7     | 8     | 9     | 10    | 11    | 12   | 13    | 14    |
|------------------------------------------------------|------|------|-----|-------|-------|-------|-------|-------|-------|-------|-------|------|-------|-------|
| Cuprous cyanide                                      | 60   | 60   | 75  | 75    | 75    | 90    | 60    | 90    | 45    | 45    | 67    | 45   | 45    | 45    |
| Potassium cyanide (total)                            | 102  |      | 125 |       | 83    |       | 145   | 102   | 145   | 72.5  | 72.5  | 110  | 72.5  | 72.5  |
| Sodium cyanide (total)                               |      | 81   |     | 30    | 30    |       | 30    |       | 15    |       | 15    | 30   | 15    | 15    |
| Potassium hydroxide                                  | 25   |      |     |       |       | 38    | 25    | 38    | 15    |       |       |      |       |       |
| Sodium hydroxide                                     |      | 25   |     |       |       |       |       |       |       |       |       |      |       |       |
| Free potassium cyanide                               | 15   |      | 7.5 | 7.5   | 12    |       | 15    | 15    | 7.5   | 7.5   | 13    | 7.5  | 7.5   | 7.5   |
| Free sodium cyanide                                  |      | 12   |     |       |       |       |       |       |       |       |       |      |       |       |
| Potassium sodium tartrate                            | 45   |      |     |       |       |       |       |       |       |       |       | 45   |       |       |
| Potassium gluconate                                  |      | 25   |     | 25    | 25    |       |       | 25    |       | 45    |       | 45   |       |       |
| Potassium saccharate                                 |      |      |     |       | 0.008 |       | 0.004 |       | 0.004 | 0.004 | 0.004 |      | 0.008 | 0.008 |
| Selenium diethylthio-carbamate                       |      |      |     |       |       | 0.012 |       | 0.012 |       |       |       |      |       |       |
| Tellurium diethylthio-carbamate                      |      |      |     |       |       |       |       |       |       |       |       |      |       |       |
| Lead in g./l. added as $Pb(C_2H_3O_2)_2 \cdot 3H_2O$ |      |      |     | 0.002 | 0.002 | 0.004 | 0.002 | 0.004 |       | 0.002 | 0.002 |      |       | 0.002 |
| Potassium thiocyanate                                |      |      | 15  | 5     |       |       |       |       | 0.05  |       |       |      |       |       |
| TEA N-lauryl $\beta$ -amino propionate <sup>1</sup>  | 0.15 |      |     |       |       |       |       |       | 0.05  |       | 0.05  | 0.05 | 0.05  | 0.05  |
| Sodium N-coco $\beta$ -amino propionate              |      | 0.05 |     |       |       |       |       |       |       |       |       |      |       |       |
| Sodium N-lauryl $\beta$ -amino propionate            |      |      |     |       |       |       |       |       |       |       |       |      |       |       |
| Disodium N-lauryl $\beta$ -imino dipropionate        |      |      |     | 0.10  |       |       |       |       |       |       |       |      |       |       |
| Disodium N-tallow $\beta$ -imino dipropionate        |      |      |     |       |       |       | 0.10  | 0.05  |       |       |       |      |       |       |
| Sodium N-lauryl $\beta$ -amino butyrate              |      | 0.10 |     |       |       |       |       |       |       |       |       |      |       |       |
| Temperature °C                                       | 65   | 65   | 65  | 80    | 75    | 75    | 65    | 75    |       |       |       |      |       |       |

<sup>1</sup> The abbreviation TEA refers to the triethanol-ammonium radical.

Table II

| Constituent in g./l. or Plating Condition                 | 1     | 2    | 3    | 4     |
|-----------------------------------------------------------|-------|------|------|-------|
| Cuprous cyanide                                           | 42.5  | 42.5 | 42.5 | 42.5  |
| Potassium cyanide                                         | 86    | 86   | 86   | 86    |
| Free potassium cyanide                                    | 22.5  | 22.5 | 22.5 | 22.5  |
| Potassium hydroxide                                       | 11    | 11   | 11   | 11    |
| Free potassium hydroxide                                  | 9.5   | 9.5  | 9.5  | 9.5   |
| Potassium stannate                                        | 60    | 60   | 60   | 60    |
| Potassium gluconate                                       |       | 25   | 25   | 25    |
| Potassium saccharate                                      |       | 25   |      |       |
| Potassium sodium tartrate                                 | 45    |      |      |       |
| $Pb^{++}$ in g./l. added as $Pb(C_2H_3O_2)_2 \cdot 3H_2O$ | 0.025 | 0.05 |      |       |
| Sodium N-coco $\beta$ -amino propionate                   | 0.05  |      | 0.10 |       |
| Sodium N-lauryl $\beta$ -amino propionate                 |       |      |      | 0.075 |
| Disodium N-lauryl $\beta$ -imino dipropionate             |       |      |      | 0.05  |
| Sodium N-lauryl $\beta$ -amino butyrate                   | 60    | 60   | 60   |       |
| Temperature °C                                            | 60    | 60   | 60   |       |

The cyanide alkaline type of baths for electrodeposition of copper and copper alloys which have incorporated therein the N-substituted  $\beta$ -alanines are particularly "free rinsing." Parts taken from these baths are often so free of salts and other surface material that it is not necessary to clean them before nickel plating. These  $\beta$ -alanines are exceedingly stable in cyanide baths. If there is decomposition, the products do not produce any adverse effects on the cathodic deposit and are compatible with the bath.

one  $\beta$ -alanine selected from the class consisting of compounds having the following formulae:



wherein R is an alkyl radical having from 8 to 16 carbon atoms in the chain, R' is a group selected from the class consisting of hydrogen and alkyl radicals having 1 to 4 carbon atoms, and X is a cation selected from the class consisting of hydrogen, sodium, potassium, calcium, lithium, magnesium and ammonium ions.

2. The bath as claimed in claim 1 in which the  $\beta$ -alanine is present in an amount between 0.04 and 0.09 g./l.

3. The bath as claimed in claim 2 wherein the R radical has from 12 to 14 carbon atoms, the R' group is hydrogen, and the cation is the sodium ion.

4. The bath as claimed in claim 2 wherein the R radical has from 12 to 14 carbon atoms, the R' group is hydrogen, and the cation is the potassium ion.

5. The bath as claimed in claim 2 in which the  $\beta$ -alanine is sodium N-coco  $\beta$ -amino propionate.

6. The bath as claimed in claim 2 in which the  $\beta$ -alanine is sodium N-lauryl  $\beta$ -amino propionate.

7. The bath as claimed in claim 2 in which the  $\beta$ -alanine is triethanol ammonium N-lauryl  $\beta$ -amino propionate.

8. The bath as claimed in claim 2 in which the  $\beta$ -alanine is sodium N-lauryl  $\beta$ -amino butyrate.

9. In a method of electrodepositing a metal selected from the class consisting of copper and copper base alloys, the step of depositing said metal from an alkaline-cyanide bath comprising copper cyanide, free cyanide, and between 0.01 g./l. and 0.2 g./l. of at least one  $\beta$ -alanine selected from the class consisting of compounds having the following formulae:



wherein R is an alkyl radical having from 8 to 16 carbon atoms in the chain, R' is a group selected from the class consisting of hydrogen and alkyl radicals having 1 to 4 carbon atoms, and X is a cation selected from the class consisting of hydrogen, sodium, potassium, calcium, lithium, magnesium and ammonium ions.

10. A method as claimed in claim 9 in which the  $\beta$ -alanine is present in an amount between 0.04 and 0.09 g./l.

11. A method as claimed in claim 10 in which the  $\beta$ -alanine has the general formula



the R radical has from 12 to 14 carbon atoms, R' is hydrogen, and the cation is the sodium ion.

12. A method as claimed in claim 10 in which the  $\beta$ -alanine has the general formula



5 the R radical has from 12 to 14 carbon atoms, R' is hydrogen, and the cation is the potassium ion.

13. A method as claimed in claim 9 in which the  $\beta$ -alanine is sodium N-coco  $\beta$ -amino propionate.

14. A method as claimed in claim 9 in which the  $\beta$ -alanine is sodium N-lauryl  $\beta$ -amino propionate.

15. A method as claimed in claim 9 in which the  $\beta$ -alanine is triethanol ammonium N-lauryl  $\beta$ -amino propionate.

16. A method as claimed in claim 9 in which the  $\beta$ -alanine is sodium N-lauryl  $\beta$ -amino butyrate.

17. In an alkaline cyanide copper electroplating bath, the improvement which comprises the addition of a compound of the formula



20 wherein R is an alkyl radical having from 8 to 16 carbon atoms, n is from 2 to 3, and X is a cation selected from the class consisting of hydrogen and sodium, the amount of said compound being at least 0.01 g./l.

25 **References Cited** in the file of this patent

## UNITED STATES PATENTS

|              |               |               |
|--------------|---------------|---------------|
| 2,255,057    | Holt          | Sept. 9, 1941 |
| 2,876,178    | McCoy         | Mar. 3, 1959  |
| 30 2,881,122 | Foulke et al. | Apr. 7, 1959  |